

Dec. 8, 1936.

J. M. HUGHES ET AL

2,063,677

METHOD OF ROLLING COPPER STRIPS AND THE LIKE

Filed April 11, 1932

2 Sheets-Sheet 1



Fig. 1



Fig. 2



Fig. 3



Fig. 4

Inventors  
John M. Hughes  
Joseph H. Carter  
Eustace E. Reagle

By  
Please and Bishop Attorneys

Dec. 8, 1936.

J. M. HUGHES ET AL

2,063,677

METHOD OF ROLLING COPPER STRIPS AND THE LIKE

Filed April 11, 1932

2 Sheets-Sheet 2



Fig. 5



Fig. 6



Fig. 7



Fig. 8

Inventors  
John M. Hughes  
Joseph H. Carter  
Eustace E. Reagle

Please and Bishop Attorneys

## UNITED STATES PATENT OFFICE

2,063,677

METHOD OF ROLLING COPPER STRIPS  
AND THE LIKE

John M. Hughes and Joseph H. Carter, Youngstown, Ohio, and Eustace E. Reagle, Sharon, Pa., assignors to Sharon Steel Corporation, a corporation of Pennsylvania

Application April 11, 1932, Serial No. 604,510

5 Claims. (Cl. 80—60)

The invention relates to the art of rolling copper or brass or similar non-ferrous metal strips and the like from large ingots, and more particularly to the rolling of copper and the like to produce coiled strips and the like having characteristics superior to the characteristics of such strips produced in accordance with standard practice.

Cold rolled copper strips have been made from cake copper cast in various sizes, say from 10 8" x 24" x 1.25" to 14" x 28" x 2" weighing from 80 to 260 pounds. The copper cakes are scalped and sometimes pickled and are then passed through cold rolls to about fifty percent reduction after which they are annealed and pickled. Cold 15 rolling followed by annealing and pickling after each fifty percent reduction is continued until the required finished gauge is obtained.

Cold rolled copper strips have been made from cake copper cast in larger sizes having thicknesses 20 of from three to four inches and weighing about 500 pounds. These larger cakes are scalped and sometimes pickled, and are then hot rolled on ordinary mills to say 0.125" to 0.187" in thickness, and are then coiled, the coils weighing approximately 25 500 pounds. The coiled strips are then cold rolled to say 0.005" with one or more anneals and pickles.

The hot rolling has been performed in accordance with prevailing practice on an ordinary hot 30 mill of either the pullover type or the reversing type, and the hot rolled product is usually somewhat brittle and has cracked edges, which require slitting or trimming before using.

In accordance with standard practice, cold rolling 35 is performed on standard two high mills with hand or power screw downs, the use of which requires annealing and pickling operations after each fifty percent reduction; or cold rolling may be carried out on a "Steckel mill" enabling greater 40 reductions and fewer anneals and pickles.

However, when long length strips are made by hot and cold rolling and annealing in accordance with standard practice, the cold rolled strips are not only very brittle and will not stand sharp 45 bending without cracking, but also have such cracked edges as to require their edges to be trimmed before tubes or other products can be made from the same.

Moreover, strips made even from 500 pound 50 cakes do not have sufficient length to be economically cold rolled on a "Steckel mill", so that two or more of the same are frequently joined together end to end for being cold rolled on a "Steckel mill."

55 It is therefore a principal object of the present

invention to roll copper strips and the like with increased production, and with a reduction in manufacturing costs, and to obtain a product having improved qualities and characteristics.

It is also an object of the present invention to 5 roll hot roll copper strips and the like in extremely long lengths to form coils weighing 1000 pounds and upwards, which may be economically cold rolled on a "Steckel mill" without splicing.

It is likewise an object of the present invention 10 to roll copper strips and the like by hot and cold rolling so that a finished product may be obtained without, in most instances, requiring any annealing operations to be performed.

It is a further object of the present invention to 15 roll copper strips and the like, so that the resulting hot or cold rolled product has edges which are so true and solid as to require little if any trimming to be performed; and so that the resulting cold rolled product is so ductile that it may be 20 bent with a flat fold with or parallel to the grain without cracking the folded edge.

Moreover, it is an object of the present invention to roll copper strips and the like directly from large cast ingots weighing, say, 8000 pounds, and obtain a much greater yield of finished material 25 than has been obtained by previous practice.

Furthermore it is an object of the present invention to roll copper strips and the like directly from large cast ingots weighing, say, 8000 pounds 30 in much less time and with much less labor than are required by standard practice.

Likewise it is an object of the present invention to eliminate the continual manual handling and rehandling of copper coils and the like, which 35 accompanies the present practice of hot and/or cold rolling of copper strips and the like.

And finally, it is an object of the present invention to roll copper strips and the like and avoid the present hot and cold rolling difficulties; and 40 to obtain a product in which undesirable characteristics are eliminated.

We have discovered that the above and other objects can be accomplished by our improvements in the art of rolling copper strips and the like 45 wherein cast copper ingots and the like, which may be 20" x 20" x 5"—6", weighing about 8000 pounds, are heated to between 1500° F. and 1700° F., say 1550° F., are then hot rolled by a plurality of passes preferably on a two-high reversing 50 blooming mill, in some 2 to 3 minutes, and are then end cropped and sheared to form blooms. The blooms are then continuously rolled on a plurality of reducing and edging mills, and are sheared to form slabs and the like of any de- 55

sired dimensions and weight, which may be say 2 inches thick by 6 inches wide by 30 feet long weighing approximately 1250 pounds.

The slabs are then reheated to between 1400° F. and 1700° F., say about 1500° F., are then reduced in a continuous hot mill, including some edge rolling, to a bar or strip or sheet of any desired dimensions, which may have a thickness of say 0.1 inches more or less, all in approximately one minute or less or before the strips have cooled below a proper hot rolling temperature, and the strips are then coiled. The finishing temperature of the strips is between 800° F. and 1300° F., say about 1100° F., and the coiled strips weigh approximately 1250 pounds, according to the size of the slabs from which they are rolled.

The equipment for continuously hot rolling the slabs to form strips and the like may include a series of some eleven stands of hot rolls, and some four sets of vertical axis edge rolls may be located, one before the first stand of hot rolls, one after the second stand of hot rolls, one after the fourth stand of hot rolls and one after the fifth stand of hot rolls. The rolls are preferably operated at a speed which will pass any given portion of the strip through the series of rolls in approximately thirty seconds, so that the entire strip will pass through the continuous hot rolling mill in approximately one minute or less in order that the hot roll reduction may be performed before the strip has cooled below a proper hot rolling temperature.

We have discovered that hot rolled strips made in accordance with the present invention have true or solid edges and that they are considerably more ductile than hot rolled strips made by prevailing practice.

It is known that copper has higher ductility at high temperatures in an oxidizing atmosphere, and this characteristic may possibly account for the improved characteristics of the hot rolled product made in accordance with the present invention, because so much work is performed upon the metal when the same has high ductility at high temperatures in an oxidizing atmosphere in a short space of time, i. e., reduction from a 20" x 20" ingot to 0.1 inch thick strip with an effective rolling time of approximately six or seven minutes.

Moreover, the high ductility and lack of brittleness of the hot rolled product, made in accordance with the present invention, may also possibly arise from the fact that little if any copper oxide forms on the surfaces of the strip; because the hot work is performed so quickly that the oxide does not have time to form, and because the ratio of surface to volume of the large ingots and slabs handled is much less than a similar ratio which might be established with respect to cakes rolled in accordance with prevailing practice.

The hot rolled coiled strips may then be cold rolled to a thickness of 0.005 inch or lighter without any annealing, and a much greater yield is obtained than has been obtained by previous practice. Moreover the edges of the cold rolled product are so true or solid as to require little, if any, trimming, and the cold rolled product is so ductile that it may be bent with a flat fold 70 with or parallel to the grain without cracking the folded edge.

A combination and general arrangement of commercial apparatus, which has been successfully utilized in carrying out the new art of 75 rolling copper strips and the like, is diagram-

matically illustrated in the accompanying drawings, forming part hereof, in which:—

Figure 1 is a plan view of a soaking pit, a blooming mill, a shear, and a crop pit, together with intervening conveyors, for reducing ingots to blooms by hot rolling operations.

Fig. 2 is a side elevation of the same;

Fig. 3 is a plan continuation view of the hot rolling apparatus, including a tandem series of five hot roll stands with edge roll stands located 10 before the first and third hot roll stands, for rolling the blooms to slabs; a shear for cropping off ends or cutting the slabs to desired lengths; a plurality of hot beds; a stand of pinch rolls; and a delivery table; together with intervening 15 conveyors;

Fig. 4 is a side elevation of the same;

Fig. 5 is plan continuation view of the hot rolling apparatus, including a charging conveyor, a slab heating furnace, a pusher, a shear, a tandem series of some eleven continuous roughing and finishing hot roll stands with some four edging roll stands, and a delivery conveyor;

Fig. 6 is a side elevation of the same;

Fig. 7 is a plan continuation view of a conveyor, vibrators, apron conveyors, pinch rolls, shears, reels, conveyors, and delivery stations; and

Fig. 8 is a side elevation of the same.

Similar numerals refer to similar parts throughout the drawings.

For carrying out the improved art of rolling copper strips and the like, a cast copper ingot, which may be 20" x 20" x 5"—6", weighing about 8000 pounds, may be delivered to the soaking pit 10 wherein it is heated to between 1500° F. and 1700° F., say 1550° F., and is withdrawn therefrom and passed by a conveyor 11 to a two-high reversing blooming mill 12 wherein it is given a plurality of passes to break the ingot 40 down to bloom size.

The bloom is carried from the blooming mill 12 by a conveyor 13 to a shear 14 for cropping irregular ends of the bloom and for cutting the same into convenient or desired bloom lengths, 45 the end crops being received by the crop pit 15.

A conveyor 16 receives the blooms for delivering them to the continuous hot rolling mill 19, which may preferably include tandem series stands of some five hot rolls 19a, 19b, 19c, 19d and 19e, and edge rolls 19a' and 19c' located ahead of the first and third stands of hot rolls 19a and 19c wherein the blooms are rolled by continuous single ply passes to slab size. The slabs are then delivered to the shear 20 and cut to convenient slab lengths, say two inches thick by six inches wide by thirty feet long, each weighing approximately 1250 pounds, or the same are rolled and cut to other desired sizes according to the desired dimensions of the final product to be 60 produced. The slabs are then delivered by a conveyor 21 to hot beds 22, whence pinch rolls 23 may deliver the same to the delivery table 24.

The slabs are then transferred from the table 24 to a charging conveyor 25 and charged into a heating furnace 26 wherein they are reheated to between 1400° F. and 1700° F., say about 1500° F., and are delivered from the heating furnace 26 by pusher 27 to continuous roughing and finishing mills indicated generally at 28 and 29 respectively.

The roughing mill may include a shear 28a, some five continuous hot roll stands 28b, 28c, 28d, 28e and 28f, with edging mill stands 28b', 28d', 28f' and 28g' located before the first, third and 75

fifth hot roll stands and after the fifth hot roll stand; and the finishing mill 29 may include some six continuous hot roll stands 29a, 29b, 29c, 29d, 29e and 29f.

5 The slabs are passed continuously through and reduced by single ply passes in the immediately succeeding operations of the successive stands of the mills 28 and 29 to a strip having a thickness of say 0.1 inch more or less, all in approximately one minute or less, and before the strip has cooled below a proper rolling temperature of between 800° F. and 1300° F., say about 1100° F.

The hot rolled strip is then passed to one of the vibrators 30, along an apron conveyor 31, through pinch rolls 32 to a reel 33 for the purpose of being coiled, the shear 34 being utilized for cutting off irregular ends of the strip, after which the coils are passed along conveyors 35 to a delivery station 36.

20 The hot rolled strip coils may then be passed through cold rolls and rolled to approximately 95 percent reduction, say from 0.1" to 0.005" without any annealing, and then coiled.

The hot rolled strips thus made have true or solid edges and are considerably more ductile than hot rolled strips made by prevailing practice; and a much greater yield is obtained than has been obtained by previous practice. Moreover, the edges of the cold rolled strips are so true or solid as to require little, if any trimming, and the strip is so ductile, without annealing, that it may be bent with a flat fold without cracking the folded edge. In other words, the hardness of the finished materials is not increased so much and ductility is not decreased so much by carrying out the present process as occurs in carrying out prevailing practice.

40 The term "copper strips" utilized in the appended claims is intended to refer to copper, or brass, or similar non-ferrous metals; and to strips, or to sheets and the like, which may be sheared from the strips.

45 It is not intended to limit the scope of the present invention to the particular temperatures mentioned, because various brasses or similar non-ferrous copper alloys require different hot rolling temperatures lower or higher than the particular temperatures referred to.

Nor is it intended to limit the scope of the 50 present invention to the particular rolling times referred to, because certain alloys may require slower rolling; although one of the essential features of the present invention involves the rapid hot rolling of copper or brass or similar non-ferrous metals to extreme reductions of say approximately 95 percent by continuous successive deep drafts.

55 And finally, it is not intended to limit the scope of the present invention to the particular ingot sizes, or to the particular thicknesses of

hot rolled or cold rolled strips referred to, because these sizes and thicknesses may be varied in accordance with the nature of the product to be produced.

We claim:—

1. The method of rolling a copper strip which includes heating a slab to rolling temperature, continuously reducing and edge rolling the same to form a hot rolled strip before the strip has cooled below a proper hot rolling temperature, 10 and then cold rolling the hot rolled strip to approximately 95 percent reduction to form a ductile cold rolled strip without annealing the same.

2. The method of rolling a copper strip which includes heating a 2" thick slab to rolling temperature, continuously reducing and edge rolling the same to form a 0.1" thick hot rolled strip before the strip has cooled below a proper hot rolling temperature, and then cold rolling the hot rolled strip to a thickness of approximately 20 0.005" to form a ductile cold rolled strip without annealing the same.

3. The method of rolling a copper strip which includes heating a slab to rolling temperature, continuously reducing and edge rolling the same 25 to form a hot rolled strip before the strip has cooled below a proper hot rolling temperature and coiling the same, cold rolling the hot rolled strip to approximately 95 percent reduction to 30 form a ductile cold rolled strip without annealing the same, and then coiling the same.

4. The method of rolling copper strips which includes heating an ingot to rolling temperature, breaking down the ingot by rolling to form 35 blooms, continuously rolling the blooms to form slabs, heating the slabs to rolling temperature, continuously reducing and edge rolling the slabs to form strips each weighing 1000 pounds and upwards by single ply passes before the strips 40 have cooled below a proper hot rolling temperature, coiling the hot rolled strips, and then cold rolling the hot rolled strips to form ductile cold rolled strips without annealing the same.

5. The method of rolling copper strips which 45 includes heating an ingot to rolling temperature, breaking down the ingot by rolling to form blooms, continuously rolling the blooms to form slabs, heating the slabs to rolling temperature, continuously reducing and edge rolling the slabs 50 to form strips by single ply passes before the strips have cooled below a proper hot rolling temperature, coiling the hot rolled strips, and then cold rolling the hot rolled strips to form 55 ductile cold rolled strips without annealing the same.

JOHN M. HUGHES.

JOSEPH H. CARTER.

EUSTACE E. REAGLE.

60